

Patented Oct. 23, 1923.

1,471,410

# UNITED STATES PATENT OFFICE.

SPENCER B. NEWBERRY, OF CLEVELAND, OHIO; ANDREW W. NEWBERRY EXECUTOR OF SAID SPENCER B. NEWBERRY, DECEASED, ASSIGNOR TO MEDUSA CONCRETE WATERPROOFING COMPANY, OF CLEVELAND, OHIO, A CORPORATION OF MAINE.

## PROCESS OF MAKING WATERPROOFING FOR CONCRETE AND THE PRODUCT THEREBY PRODUCED.

No Drawing.

Application filed July 2, 1921. Serial No. 482,253.

*To all whom it may concern:*

Be it known that I, SPENCER B. NEWBERRY, a citizen of the United States, and resident of Cleveland, county of Cuyahoga, 5 State of Ohio, have invented certain new and useful Improvements in Processes of Making Waterproofing for Concrete and the Product Thereby Produced, of which the following is a specification.

10 This invention relates to a process for making waterproofing for concrete and the product thereby produced. It is designed to more perfectly prevent the penetration of water into the concrete through surface voids or pores than has been possible by coatings heretofore used. The novel features will be understood from the following description and claims.

Integral waterproofing for rendering cement concrete impervious to water is commonly made, as described in Patent No. 851,247, issued to me April 7, 1907, by combining fatty acids with lime by heat and grinding the resulting lime compound of fatty acids to fine powder. The degree of waterproofing effect produced by the material depends to a great extent on its fineness of subdivision, since the function of the waterproofing is to coat the surfaces of the voids or pores of the concrete and to exert a water-repellent action which prevents absorption or penetration of water into the mass. The method of preparation of the waterproofing commonly employed is to melt the fatty acid by heat and to stir in sufficient lime to bring the fatty acid into complete combination, then after cooling, to grind the solid lime compound, with the addition of a further quantity of lime in hydrated form, to fine powder. Another method, as described in Patent No. 851,247, is to slake quick lime and add fatty acid, thus effecting the combination by the heat of the slaking of the lime, and finally to dry and grind the product.

A long series of careful tests have demonstrated that the employment of heat in combining fatty acids with lime greatly injures the water-repellent effect of the product, and that if this combination takes place in the cold, that is without sensible rise in temperature above that of the atmosphere, a product of almost molecular fineness, pos-

sessing waterproofing qualities far beyond those of any materials hitherto known, is 55 obtained. If two blocks of concrete are prepared, one containing the best waterproofing now on the market, and the other a waterproofing of the same composition but prepared by the cold method, the latter will 60 be found to absorb only one-fourth to one-third as much water as the former. This marked difference is doubtless largely due to the extreme fineness of the cold-prepared material, a fineness which it is practically 65 impossible to reach by any method of grinding in the case of waterproofing prepared by a process in which heat, even as high as the boiling point of water, is employed. Even with equal fineness it will be found 70 that waterproofing containing fatty acids is greatly injured in its water-repellent qualities by exposure to very moderate heat, and that greatly superior water-repellent qualities are possessed by a compound which 75 has not been exposed to a temperature greatly exceeding that of the atmosphere.

The method of making the fatty acid compound without the use of heat, which I have found most economical and efficient, is to 80 bring the fatty acid, in lump or liquid form, into contact with hydrated lime and to subject the mixed materials to a stirring or grinding operation. I prefer to use solid fatty acid, known as stearic acid, but containing also palmitic and oleic acids, but 85 commercial red oil, consisting chiefly of oleic acid, may also successfully be employed. When the fatty acids come into contact with the lime combination takes place at once 90 without noticeable rise in temperature, with the formation of a lime compound in almost infinitely fine subdivision. The only grinding action necessary therefore, is one which will detach from the lumps or masses of 95 fatty acid the coating of lime compound formed on them, and thus bring the surfaces of fatty acid into contact with fresh portions of lime, until all the materials are 100 fully combined and disintegrated. Prolonged agitation in a pug-mill will accomplish this result; but I have found that time is saved and the cost of the operation reduced by use of a swing-hammer or impact pulverizer of the well known Williams or 105 Raymond type, combined with an air sepa-

rator. A tube mill, with or without air separation, may also be used. The fineness of the product should be such that at least 95 per cent will pass a 200 mesh sieve. By 5 careful manufacture it is possible to reach such fineness that practically 100 per cent will pass 200 mesh.

In place of hydrated lime, any other calcium compound which will combine with 10 fatty acids and will not evolve sensible heat when treated with water, may be used. Such compounds of calcium are the basic silicates and aluminates which are the principal constituents of hydraulic cement. Wa- 15 terproofing compound which falls within the scope of this application may therefore be made by mixing fatty acids with Portland or natural cement and stirring or grinding the mixture till a homogeneous, finely-di- 20 vided product is obtained.

What I claim as new and desire to secure by Letters Patent is—

1. Process of making waterproofing by 25 mixing fatty acid with hydrated lime and stirring the mixture without heating it above ordinary atmospheric temperature, until the product becomes a homogeneous finely-divided powder.

2. Process of making waterproofing by 30 mixing fatty acid with hydrated lime and pulverizing the mixture without heating it above ordinary atmospheric temperature, to an impalpable powder.

3. Process of making waterproofing by 35 mixing 10 to 25 parts fatty acid with 100

parts hydrated lime and pulverizing the mixture, without heating it above ordinary atmospheric temperature, to an impalpable powder.

4. Process of making waterproofing by 40 mixing fatty acid with hydrated lime and pulverizing the mixture, without heating it above 212 degrees F., to an impalpable powder.

5. A waterproofing powder consisting of 45 fatty acids and hydrated lime in combination and fine subdivision, which at no stage of its manufacture has been heated above ordinary atmospheric temperature.

6. A waterproofing powder consisting of 50 fatty acids and hydrated lime in combination and fine subdivision, which at no stage of its manufacture has been heated above 212 degrees F.

7. Process of making waterproofing by 55 mixing fatty acid with basic calcium compounds which do not evolve sensible heat on treating with water, and pulverizing the mixture without heating it above the ordinary atmospheric temperature, to an im- 60 palpable powder.

8. Process of making waterproofing by 65 mixing fatty acid with basic calcium compounds which do not evolve sensible heat on treating with water, and pulverizing the mixture without heating it above 212 degrees F., to an impalpable powder.

In testimony whereof I hereunto affix my signature.

SPENCER B. NEWBERRY.